

Aug. 14, 1934.

V. BOSSO ET AL

1,970,273

PRODUCTION OF MATERIALS, DECORATIVE ARTICLES, AND PROTECTING LININGS OR  
THE LIKE, BY THE TRANSFORMATION OF FIBROUS CELLULOSE MATERIALS

Filed July 9, 1932

2 Sheets-Sheet 1



*Fig. 1.*

*Fig. 4.*



*Fig. 2.*

INVENTORS:  
V. Bosso  
N. Silvestrini  
F. Sacchi  
BY *Marks & Clark*  
ATTORNEYS.

Aug. 14, 1934.

V. BOSSO ET AL. 1,970,273  
PRODUCTION OF MATERIALS, DECORATIVE ARTICLES, AND PROTECTING LININGS OR  
THE LIKE, BY THE TRANSFORMATION OF FIBROUS CELLULOSE MATERIALS  
Filed July 9, 1932 2 Sheets-Sheet 2



*Fig. 3.*



*Fig. 5.*



BY *Marks & Clark*  
ATTORNEYS.

Patented Aug. 14, 1934

1,970,273

# UNITED STATES PATENT OFFICE

1,970,273

## PRODUCTION OF MATERIALS, DECORATIVE ARTICLES, AND PROTECTING LININGS OR THE LIKE, BY THE TRANSFORMATION OF FIBROUS CELLULOSE MATERIALS

Valentino Bosso, Nicolo Silvestrini, and Francesco Sacchi, Torino, Italy, assignors to Guido Botta, Paris, France

Application July 9, 1932, Serial No. 621,644  
In France November 16, 1931

16 Claims. (Cl. 92—40)

The invention relates to the production of materials for making decorative articles and protective linings or the like.

It is known that, in the production of objects of a decorative nature, or of articles serving for lining and protecting walls, floors, ceilings, furniture and the like, use is sometimes made of sheets, boards, mouldings, or the like, which are formed by assembling, drying and compressing fibrous cellulosic materials, or by other analogous means.

Thus these fibrous materials are commonly employed in the form of sheets of considerable thickness.

15 It is known that the fibres composing fibrous cellulosic materials are capable of agglomerating and forming a continuous material, possessing strength simply by using water as the sole agglomerating agent.

20 The water separates the fibres in proportion to the volume of water employed. The present invention is in part based on the observation that the degree of agglomeration of the fibres being treated may be regulated as desired by regulating the quantity of water.

The invention is also based upon the observation that the marbling and veins which are noticeable, for example, in sheets of crude cellulose, such as those that come off paper machines, (see Figure 1 of the drawings) can be exploited from the decorative point of view, on account of the non-uniform color-absorbing capacity or on account of the simple differences in natural color or tone, which they adopt when they undergo 30 the treatment effected during the second stage of the process set forth below.

The marbling, veins or streaks as they generally occur, are not sufficiently pronounced, nor sufficiently decorative. This desired decorative 40 appearance can be obtained in accordance with this invention by accentuating and exaggerating the appearance and shape of the marbling, veins, etc.

45 It is an object of this invention to provide a process which causes marbling and veining to be produced artificially.

The methods of carrying out this process may differ depending on whether they are applied to fibrous boards in the wet state, in the dry state, or during drying treatment; but essentially they are all based upon an exaggeration of the mechanical effects which normally tend to produce these breaks in continuity.

55 The present invention provides a method for producing decorative materials from cellulose

fibres in which we can regulate or control the lateral vibrations applied to the screen of a paper machine while regulating the water supply, so as to effect an irregular distribution of the fibres in the sheet to obtain marbling, veins 60 and the like, good results having been obtained by doubling the vibrations per minute as compared with paper making practice, while keeping the speed of longitudinal movement of the screen constant. 65

The adjustment of the water supply may be effected either by employing an excess of water, or in adding collagenous materials such as a decoction of linseed to the water employed in the process, for the purpose of making the mass more 70 viscous. The linseed makes the water employed in the process definitely colloidal in nature, and very viscous, so as to render the drying operation difficult. Thus, the paste or pulp which arrives charged with water, particularly in the thicker 75 parts which have been produced in the form of longitudinal thickenings by the action of the exaggerated vibrations above referred to, is forced out under the press very suddenly where the veins are situated, and this increases the size of the 80 openings at these points.

When the sheet is dried the veins may be still further accentuated if the sheet is wound upon itself, and if, for example, it is subjected to a twisting action at one end in the direction of the 85 axis upon which it is wound, while keeping the other end fixed; or if it is subjected to a crumpling or creasing action carried out by hand, or again, if the continuous sheet is made to pass between cylinders which are not uniformly round, but comprise irregularities of a positive nature on one cylinder, and of a negative nature on the other cylinder with the object of producing this crumpling or creasing artificially. 90

Finally, in certain cases the boards may be 95 subjected to the action of a preliminary bath in a solution of an astringent material which by rapid drying creases or lines the boards.

The second stage of our improved method comprises a gumming operation in which we utilize 100 animal gelatine.

This bath is characterized by the fact that a substance containing the group  $\text{SiO}_2$  e. g. sodium silicate or silicic acid is incorporated in the gelatine solution. This gives the gumming solution 105 a special property, the finished product acquiring increased thickness and compactness and increased waterproofness.

According to our invention above mentioned substances may be incorporated in the gumming

baths, either separately in aqueous solutions, or by soaking the paper and the fabric to be gummed previously with the solutions, or by causing these substances to be formed or liberated in the bath itself.

5 The following mode of procedure is given by way of example only, and is not limiting in any way.

10 The gelatine bath is prepared by dissolving 25 kilograms of very fine dry gelatine in 100 litres of water. The temperature is raised to 50° C., and if desired, as far as 70° C. When all the gelatine is dissolved a quantity of sodium silicate is added, which may vary in amount from 100 grs. to 15 500 grs. and then 200 grs. of aluminium sulphate or 250 grs. of ordinary alum are added.

It is preferable to add these salts after they have been dissolved in water.

20 It is also possible to vary the order in which the substances are added, and add the alum or aluminium sulphate before the silicate.

In place of sodium silicate, potassium silicate and other silicates may be added, or silicic acid in a suitable form.

25 The gumming bath after successive periods of agitation and rest is utilized in the usual way, and the material to be treated may be made to pass through it in sheets, or in continuous rolls, according to the form in which it is employed.

30 In order to increase the stiffness of the finished material it is sufficient simply to increase the proportion of the silicates to about 500 grs. or more, the remainder of the operation remaining unchanged as described above.

35 As soon as the material has left the bath it is allowed to dry gradually in a chamber at normal temperature (about 20° C.) and with a simple current of air for a period of 24 hours.

40 In addition to the foregoing applicants have found that if the sheet of material, after leaving the gumming bath, is subjected to a current of cold air at a temperature around 5 to 10° C. the state of gel which is formed tends to improve the technical properties and the strength of the sheet. The latter when subsequently fixed or tanned behaves better than when treated at ordinary temperature, that is to say, at 20° to 30° C. because with the latter temperatures a wide dispersion of the material occurs in the connection between the fibres which compose the sheet 45 itself.

50 Subsequently the sheets are treated to a fixing and hardening or tanning action in a suitable bath, such as a hot gaseous formaldehyde bath, or a cold dilute formaldehyde bath; or a hot 10% bath of potassium chromate, to which is added 1% of castor oil emulsion; or a chromic acid bath; or other suitable baths. The material resulting from the action of the gumming bath is more homogeneous from the molecular and chromatic point of view when the drying action is carried out uniformly and naturally.

55 Naturally the invention also comprises modifications in the composition of the gumming bath, to which, in addition to the materials indicated above, other plastifying substances may be added, such for example as a rational proportion of glycerine etc.

60 If salts of the alkali or alkaline earth metals (e. g. K, Na, Ca) are added to the gelatine bath, with other salts, preferably halides, or heavy metals, salts such as salts of tin, aluminium, copper etc., fatty bodies may be readily incorporated in the form of insoluble soaps of those substances 65 that are saponifiable and which have an added

waterproofing action while fatty or waxy substances which do not saponify, are distributed in the mass in the form of an emulsion.

When the material has been soaked by immersion in the gelatine solution it is desirable that it be subjected to supplementary coagulating, or waterproofing action, by a known process as indicated above, that is to say, by means of formaldehyde, potassium chromate, chromic acid, or by similar substances.

80 The impregnation of the cellulose material whether in the form of cardboards, wood pulp, cotton pulp etc., is considerably improved when these materials or articles have been previously subjected to a softening treatment by means of gases or vapours of a suitable nature.

85 90 Applicants have found that as a result of this softening action the materials treated can absorb a much greater quantity of the gumming bath, and retain a greater quantity of gelatine.

95 On account of this more intense gelatinization the finished product is improved by the fact that a more intimate connection exists between the gelatine and the fibres, and consequently the outer layer of gum has a greater thickness. When 100 the cellulose material is to be immersed in solutions of animal gelatine acetic acid vapours at high temperature are most effective for producing this preliminary softening. One method of applying the acetic acid vapours may consist in 105 enclosing the cellulose materials in any suitable form, such as cardboard, linters etc., in containers or casings having a fluid-tight closure. These containers are then put into communication with a vacuum machine.

110 When the maximum possible vacuum has been obtained the communication between the vacuum machine and the container is cut off, and the latter is put into communication with an autoclave apparatus containing acetic acid which has been 115 brought to a state of superheated vapour. Approximately a quarter of an hour after the communication has been established the atmosphere containing the cardboard, linters etc., has generally been completely saturated. This communication is then cut off, and the cardboards and the linters are left for 3 to 4 hours in this saturated atmosphere.

120 Finally, air under pressure is admitted at one side of the receptacle. This air passes out at 125 the other side of the receptacle and carries away the residue of the acetic vapours.

130 Cardboards and linters etc., thus prepared, are ready for treatment in one of the gumming baths described above. Subsequently, after a uniform drying they pass into a tanning or hardening bath as described for transforming these incorporated materials into a new material, having a new form and character.

135 In the accompanying drawings the invention is illustrated, and

Figure 1 shows a plan view of a portion of a continuous sheet of cellulose as it has left the paper machine;

Fig. 2 shows the same sheet after it has been 140 submitted to torsion or twisting;

Fig. 3 shows the sheet in Fig. 2 after it has again been flattened out;

Fig. 4 shows a similar sheet of cellulose which has been subjected to a mechanical crumpling 14 and creasing; and

Fig. 5 shows in end view a pair of cylinders 10 and 11, the surfaces of which are provided with complementary ribs 12 and grooves 13 and between which is passed a sheet 14 of cellulose for 15

accentuating marbling or configuration on the surface of the sheet.

These examples have been given simply for the purpose of indicating modes of carrying the process into effect. It is clear that the field of use of the invention is not limited to this mode of operation, nor to the use of acetic acid, but that it comprises all the modifications of the softening and fixing treatment by gases or vapours, as set forth in the preamble to the specification.

We claim:

1. Process for the production of decorative materials from cellulose fibers, consisting in forming a sheet from a suspension of said cellulose fibers, in producing as the sheet is being formed an accentuated irregular distribution of the fibers in the sheet for obtaining marbling, veins and the like consisting of sheet portions in which the fibers are thickened or more closely set, in treating the sheet in a gumming bath comprising a solution of gelatine, to which a substance containing  $\text{SiO}_2$  has been added, and thereupon in a fixing bath containing formaldehyde and castor oil.

2. Process for the production of decorative materials from cellulose fibers, consisting in forming a sheet on a paper making machine from a dilute solution of said fibers to which a linseed decoction has been added while vibrating the wire of the machine sufficiently to produce an irregular accentuated distribution of the fibers for the purpose of obtaining marbling, veins and the like, treating the sheet thus formed in a gumming bath comprising a gelatine solution to which a substance containing  $\text{SiO}_2$  has been added and in treating the sheet in a fixing bath containing formaldehyde and castor oil.

3. Process for the production of decorative materials from cellulose fibers, consisting in forming a sheet on a paper machine from a suspension of said cellulose fibers, in drying the sheet, in winding and twisting said sheet so as to obtain thereon a plurality of zones having a smaller resistance to penetration of a liquid, in treating said sheet in a gumming bath comprising a gelatine solution to which a substance containing  $\text{SiO}_2$  has been added and thereupon in a fixing bath containing formaldehyde and castor oil.

4. Process for the production of decorative materials from cellulose fibers, consisting in forming a sheet on a paper machine from a suspension of said cellulose fibers, in treating said sheet with an astringent solution, in rapidly drying said sheet so as to cause shrinkage thereof, in winding and twisting said sheet so as to form thereon a plurality of zones having a smaller resistance to liquid penetration, in treating the sheet in a gumming bath comprising a gelatine solution to which a substance containing  $\text{SiO}_2$  has been added and in treating the sheet in a fixing bath containing formaldehyde and castor oil.

5. Process for the production of decorative materials obtained from cellulose fibers, consisting in continuously forming a sheet on a paper making machine from a dilute suspension of said fibers to which a decoction of linseed has been added, in producing as the sheet is being formed an irregular accentuated distribution of the fibers by lateral vibrations of the wire of the paper machine, for the purpose of obtaining veins, marbling and the like, in treating said sheet with an astringent solution, in rapidly drying said sheet so as to cause same to shrink and crumple, in winding and twisting said sheet so as to form thereon a plurality of zones having a smaller

resistance to liquid penetration, in treating said sheet in a gumming bath comprising a gelatine solution to which a substance containing  $\text{SiO}_2$  has been added and in treating said sheet in a fixing bath containing formaldehyde and castor oil.

80

6. Process for the production of decorative materials from cellulose fibers consisting in forming a sheet from a suspension of said fibers, in producing as the sheet is being formed an accentuated irregular distribution of the fibers in the sheet, for the purpose of obtaining veins, marbling and the like consisting of sheet portions in which the fibers are thickened, in treating the sheet in a gumming bath comprising a gelatine solution to which a substance  $\text{SiO}_2$  has been added, the  $\text{SiO}_2$  quantity not exceeding that contained in a one percent solution of silicate of sodium having the same volume as the gumming bath and in treating said sheet in a fixing bath containing potassium bichromate and castor oil.

90

7. Process for the production of decorative materials from cellulose fibers consisting in forming a sheet from a suspension of said fibers, in producing during the sheet formation an accentuated irregular distribution of the fibers in the sheet for the purpose of obtaining veins, marbling and the like, consisting of sheet portions in which the fibers are thickened, in treating the sheet in a gumming bath comprising 100 liters water, 25 kgs. gelatine, about 500 grams sodium silicate, 105 200 grams aluminium sulphate and in treating said sheet in a fixing bath.

95

8. Process for the production of decorative materials obtained from cellulose fibers, consisting in forming a sheet from a suspension of said fibers, 110 in producing as the sheet is being formed, an accentuated irregular distribution of the fibers in the sheet for the purpose of obtaining veins, marbling and the like consisting of sheet portions in which the fibers are more closely set, in subjecting the sheets thus formed to a softening operation by means of a gaseous fluid, in treating said sheet in a gumming bath consisting of a gelatine solution to which a substance containing  $\text{SiO}_2$  has been added and thereupon in a fixing 120 bath containing formaldehyde and castor oil.

115

9. Process for the production of decorative materials from cellulose fibers, consisting in forming a sheet on a paper making machine from a dilute suspension of said fibers, to which a decoction of linseed has been added, in producing an irregular accentuated distribution of the fibers by lateral vibrations of the wire of said machine, for the purpose of forming veins, marbling and the like, in subjecting the sheets thus obtained to a 130 softening operation by means of a gaseous fluid, in treating the sheet in a gumming bath comprising a gelatine solution to which a substance containing  $\text{SiO}_2$  has been added and thereupon in a fixing bath containing formaldehyde and 135 castor oil.

125

10. Process for the production of decorative materials from cellulose fibers, consisting in forming a sheet on a paper machine from a dilute suspension of said fibers, to which a decoction of linseed has been added, in producing as the sheet is being formed an irregular accentuated distribution of the fibers by lateral vibrations of the wire of said machine for the purpose of obtaining veins, marbling and the like, in treating 140 said sheet with an astringent solution, in rapidly drying said sheet so as to obtain shrinkage and crumpling thereof, in winding and twisting said sheet so as to obtain thereon a plurality of zones having a smaller resistance to liquid penetration.

145

- tion, in immersing said sheet into a dye solution so as to form thereon further veins, marbling and the like, in submitting the sheets thus obtained to a softening operation by means of a gaseous fluid, in treating the sheet in a gumming bath comprising a gelatine solution to which a substance containing  $\text{SiO}_2$  has been added, and thereupon in a fixing bath containing formaldehyde and castor oil. 80
10. 11. Process for the production of decorative materials from cellulose fibers, consisting in forming a sheet from a suspension of said cellulose fibers, in producing as the sheet is being formed an accentuated irregular distribution of the fibers in the sheet for obtaining marbling, veins and the like consisting of sheet portions in which the fibers are thickened or more closely set, in treating the sheet in a gumming bath comprising a solution of gelatine, to which a substance containing  $\text{SiO}_2$  has been added, and thereupon in a fixing bath containing formaldehyde and castor oil to which a softening substance, such as glycerine, has been added. 85
12. Process for the production of decorative materials from cellulose fibers, consisting in forming a sheet from a suspension of said cellulose fibers, in producing as the sheet is being formed an accentuated irregular distribution of the fibers in the sheet for obtaining marbling, veins and the like consisting of sheet portions in which the fibers are thickened or more closely set, in treat- 90
- 35 35 110
- 40 40 115
- 45 45 120
- 50 50 125
- 55 55 130
- 60 60 135
- 65 65 140
- 70 70 145
- 75 75 150
- ing the sheet in a gumming bath comprising a solution of gelatine to which a quantity of  $\text{SiO}_2$  has been added such that it does not exceed that contained in a one percent solution of sodium silicate having the same volume as the gumming bath with the simultaneous addition of softening substances, such as glycerine. 95
13. Decorative material which comprises a sheet of irregularly felted cellulose fibers, said fibers being disposed to form marbling, veins and like effects. 100
14. Decorative sheet material which comprises a cellulosic fibrous base in which the fibers are irregularly disposed to form marbling, veins and like effects, said base carrying an intimate reinforcing coating of a coagulated gelatinous character containing a material including the group  $\text{SiO}_2$ . 105
15. Decorative sheet material which comprises irregularly felted paper impregnated with a hardened gelatine composition containing an alkali metal silicate. 110
16. Decorative colored sheet material which comprises a member of the group consisting of paper and irregularly felted paper, impregnated with a hardened gelatinous composition containing a member of the group consisting of alkali metal silicates and silicic acid. 115
- VALENTINO BOSSO.  
NICOLO SILVESTRINI. 105  
FRANCESCO SACCHI.